

Patented Mar. 9, 1926.

1,576,179

# UNITED STATES PATENT OFFICE.

IRA H. DERBY AND CARLETON B. EDWARDS, OF INDIANAPOLIS, INDIANA, ASSIGNEES  
TO PETER C. REILLY, OF INDIANAPOLIS, INDIANA.

## PROCESS OF MODIFYING IGNITION TEMPERATURE, ETC., OF CARBONACEOUS MATERIALS AND SUCH MATERIALS.

No Drawing. Application filed August 11, 1923. Serial No. 656,914.

To all whom it may concern:

Be it known that we, IRA H. DERBY and CARLETON B. EDWARDS, citizens of the United States, residing at Indianapolis, in the county of Marion and State of Indiana, have invented certain new and useful Improvements in Processes of Modifying Ignition Temperature, Etc., of Carbonaceous Materials and Such Materials, of which the following is a specification.

Our invention relates to the manufacture of carbon compositions having relatively low ignition temperatures and high burning rates. More specifically, our invention relates to the utilization of metals or metal compounds to modify the ignition temperature and the burning rate of carbonized carbonaceous materials.

Carbonized carbonaceous substances such as petroleum coke, coal-tar coke, gas coke, and the like require heating to comparatively high temperatures to start combustion and their rates of burning are low at a given temperature. Stating the matter in slightly different language, the material has a high ignition temperature and a low burning rate.

The high ignition temperatures and the low burning rates have rendered these fuels unsuitable for use in certain industries. For example, coal-tar coke has been tested for use in the manufacture of carbonic acid (carbon dioxid), and found unsatisfactory because of its high ignition temperature.

Again, as a covering for molten lead in the steel treating lead pot, gas coke, coal-tar coke and petroleum coke are not suitable when used alone, especially in the lower temperature-range of the lead bath, though their relatively high density and low ash content are desirable characteristics. A coke igniting at a low temperature and burning more rapidly at the temperature of the lead bath offers many practical advantages in this art. Such a carbon as wood charcoal burns at a sufficiently rapid rate for use as a lead pot covering and is in common use, but has a low density and a high ash as compared with coke.

Among the substances which we have found suitable to lower the ignition temperature as well as increase the burning rate of carbonized carbonaceous materials may be mentioned the following: metallic lead;

lead carbonate; lead acetate; lead sulfide; 55 lead iodide; lead cresylate and other organic lead compounds; thallium compounds; copper oxid; barium dioxid and organic compounds of these metals easily reducible to the oxid state. It is apparent from the above that the oxid of the metal may itself be used, or that either organic or inorganic metal compounds, which easily pass into the oxid state when heated by a straight reduction or oxidation reaction or a combination thereof may be used. Some of the metal oxids appear to give better results than others and this will later be referred to in more detail. The best results have so far been attained by the use of the cresylate or 70 the oxids of lead, and the manufacture of our low igniting carbon composition and the ignition temperatures of the same will be set forth in connection with the use of the oxide of lead.

To make a coke product the following methods of manufacture may be used: (1) incorporate lead or any of the oxids of lead with pitch and carbonize or coke the mixture; (2) incorporate lead carbonate, lead acetate or any material which when heated will give the oxid, with pitch and carbonize it; (3) cause the oxid to adhere to the surface of the coke by any well-known method; and (4) dissolve a lead compound such as 85 lead cresylate, in coal-tar or pitch and distill the tar or pitch to coke. By method (4) we are able to molecularly disperse the lead throughout the coke structure thus obtaining maximum catalytic effect. To make a 90 charcoal product the following methods of manufacture may be used: (1) rub lead oxid into the pores of the charcoal; (2) saturate the charcoal with a suspension or solution of a lead compound which on heating will 95 give the oxid, and then heat to change the compound to an oxid. For example, lead acetate in water or lead cresylate in organic solvents may be employed.

It will be understood of course that the proper proportion of materials will be employed in making up the mass in bulk; thus, for producing several tons of coal-tar coke containing lead, we introduce into the still containing, say 42,000 pounds of coal tar, 105 160 pounds of lead oxide (e. g. PbO litharge). The lead oxide becomes dispersed in the tar upon heating and dissolves, thus dis-

tributing itself throughout the tar in molecular subdivision. The tar is then distilled in the usual manner until all the oils and waxes are distilled off. The coke that remains behind in the still contains the lead oxide distributed uniformly throughout its structure; in the examples given, the coke amounting to 16,000 pounds contains 1 per cent lead oxide.

10 We have also made the material in quantity by stirring lead oxide into melted coal tar pitch, or petroleum pitch, and coking the pitch. The coking process merely involves distilling off the volatile oils and obtaining 15 coke in the still as a residue.

In U. S. Patent No. 1,230,782 there is set forth the production of coke resulting from the complete distillation of coal tar. This coke is characterized by the fact that it is 20 sponge-like in appearance, amorphous, non-crystalline, dry, and when burned leaves a residue approximating two per cent composed of non-combustible matter and mineral ash. The coke is also characterized 25 by presenting when fractured a steel-gray surface upon the area of fracture, with a brilliant or glossy surface upon the walls of the depressions, pockets, or recesses appearing therein.

30 As hitherto pointed out, there is a field of great utility for a relatively dense, low ash, carbonaceous material igniting and burning at a low temperature, for example, at the temperature at which wood charcoal ignites 35 and continues to burn, the temperatures of burning of course varying in some cases, through a certain range. The coal-tar coke referred to has a satisfactory density and has, relatively speaking, a low-ash content. 40 When certain metals or metal compounds are added thereto, its ignition temperature is so depressed and the burning rate so increased that the resulting composition meets the requirements above set forth and makes 45 possible the use of the low-ash coal-tar coke in various industries. For example, we find that such coal-tar coke containing one percent of litharge is as efficient as wood charcoal and preferable from an ash standpoint. 50 In one particular sample of coal-tar coke used, an analysis showed an ash-content of 1.3 per cent. Wood charcoal usually contains from 8 to 10 per cent of ash.

55 If lead compounds are incorporated with coal before coking the coke so formed ignites at much lower temperatures than ordinary gas coke.

60 The following table indicates the depression of the ignition temperature when oxides of lead are added to low ash coal-tar coke and to wood-charcoal.

65 The ignition temperature is taken as the temperature at which appreciable combustion begins. The glow point is an indicator 05 of the ignition temperature due to the fact

that the rapidity of the combustion at the ignition temperature causes the temperature of the carbon to rise quickly to the glow point. The temperature recorded here is the ignition temperature and not the temperature of the glowing carbon.

#### Test No. I.

Air passed over 10 grams of the material at the rate of 1.3 liters per hour, in a 1" 75 glass tube heated in an electric furnace.

| Material.                                                                    | Ignition temperature. | Temperature depression. | 80 |
|------------------------------------------------------------------------------|-----------------------|-------------------------|----|
| 1. Coal-tar coke                                                             | 650                   | ° C.                    |    |
| 2. Coal-tar coke and 2% Pb <sub>3</sub> O <sub>4</sub>                       | 550                   | 100                     |    |
| 3. Coal-tar coke and 25% wood charcoal and 2% Pb <sub>3</sub> O <sub>4</sub> | 470                   | 180                     |    |
| 4. Coal-tar coke and 6% Pb <sub>3</sub> O <sub>4</sub>                       | 490                   | 160                     | 85 |

#### Test No. II.

Air passed over material at the rate of 1.3 liters per hour. Same apparatus.

| Material.                | Ignition point. | Temperature depression. | 90 |
|--------------------------|-----------------|-------------------------|----|
| Wood charcoal            | 450             | ° C.                    |    |
| Wood charcoal and 2% PbO | 310             | 140                     | 95 |

#### Test No. III.

Air passed over material at rate of 3.8 liters per hour. Same apparatus.

| Material.                                                                                     | Ignition point. | Temperature depression. | 100 |
|-----------------------------------------------------------------------------------------------|-----------------|-------------------------|-----|
| 1. Coal-tar coke                                                                              | 585             | ° C.                    | 105 |
| 2. Coal-tar coke and 2% Pb <sub>3</sub> O <sub>4</sub>                                        | 405             | 180                     |     |
| 3. Coal-tar coke and 2% PbO                                                                   | 400             | 185                     |     |
| 4. Coal-tar coke and 50% PbO (resulting from lead cresylate decomposition)                    | 330             | 255                     |     |
| 5. Coal-tar coke and 5% PbO (resulting from decomposition of lead cresylate dissolved in tar) | 395             | 190                     | 110 |

On cooling the samples of Test No. III, material No. 1, coke alone, ceased to glow (burn) at 500° C., while material No. 3 (2% PbO) ceased to glow (burn) at 260° C. Thus, PbO lowered the ignition temperature 185° C. and the temperature range through which the coke continued to burn approximately 240° C.

To show the decided difference between the lead impregnated coke and the usual coal tar coke, one piece of each was heated in the air to glowing. On removing the source of heat, the coal tar coke immediately blackened and cooled while the lead impregnated coke continued to glow, in a manner similar to the action of wood charcoal. Coke containing lead burns sufficiently rapidly on a lead bath to maintain a reducing atmosphere and a clean lead surface, whereas the usual coke

is not satisfactory because of its low rate of burning at this temperature.

Fifty (50) percent PbO in coal tar coke gives a material which may be lighted with 5 a match and will sparkle and glow brightly when blown with air, whereas ordinary coal tar coke can not be so lighted and when lighted at higher temperature is extinguished by a current of air.

10 As stated, other metals or metal compounds may be used. For example, the presence of copper oxide in coal-tar coke has an effect similar to the action of the compounds of lead but not to the same extent. 15 Fifty percent of copper oxide is necessary to approximate the results obtained with one-half to one percent of lead oxide. Using copper oxide in amounts ranging from five to ten percent only a slight depression in the 20 ignition point is obtained. We have also found that 50% barium dioxid and 50% nickel oxide are effective to depress the ignition point but their activity is decidedly lower than either that of the oxids of lead or 25 copper.

In the specification the percentages of oxids added are based on the combined weight of the coal-tar coke and the oxid. For example, two percent  $Pb_3O_4$  indicates 30 that the mix comprises 98 parts of coke and 2 parts of oxid, by weight.

Due to the great activity of small percentages of the lead compounds, also because 35 of the activity of compounds not containing oxygen, the effect is clearly a catalytic one. In the specification, then, we use the term catalyst to denote a substance which has the power of accelerating the combustion of carbon or carbonaceous material in the manner herein described in such a way as to 40 lower the ignition temperature and increase the rate of burning at a given temperature.

We claim:

1. A new article of manufacture having 45 a relatively low ignition temperature and a relatively high burning rate comprising a carbonized material and a substance containing a metal which catalyzes the combustion.

2. A new article of manufacture having a relatively low ignition temperature and a 50 relatively high burning rate, comprising a carbonized material and a metal compound which serves as a catalyst for the combustion.

55 3. A new article of manufacture having a relatively low ignition temperature and a relatively high burning rate comprising a carbonized material and a metal oxide catalyst.

60 4. A new article of manufacture having a relatively low ignition temperature and a relatively high burning rate comprising a carbonized material and from 0.1 to 50 per cent of a metal oxide catalyst.

65 5. A new article of manufacture having

a relatively low ignition temperature and a relatively high burning rate, comprising a carbonized material and an oxid of lead.

6. A new article of manufacture having a relatively low ignition temperature and a 70 relatively high burning rate comprising a carbonized material and from 0.1 to 50 per cent of an oxid of lead.

7. A new article of manufacture having a relatively low ignition temperature and a 75 relatively high burning rate comprising a carbonized material and a substance containing lead.

8. A new article of manufacture having a relatively low ignition temperature and a 80 relatively high burning rate comprising coal-tar coke and a substance containing a metal which acts as a catalyst for the carbon combustion.

9. A new article of manufacture having 85 a relatively low ignition temperature and a relatively high burning rate comprising coal-tar coke and a metal compound as a combustion catalyst.

10. A new article of manufacture having 90 a relatively low ignition temperature and a relatively high burning rate, comprising coal-tar coke and a metal oxid catalyst.

11. A new article of manufacture having 95 a relatively low ignition temperature and a relatively high burning rate comprising coal-tar coke and from 0.1 to 50 per cent of a metal oxid serving as a catalyst to accelerate the combustion.

12. A new article of manufacture having 100 a relatively low ignition temperature and a relatively high burning rate comprising coal-tar coke and an oxid of lead.

13. A new article of manufacture having 105 a relatively low ignition temperature and a relatively high burning rate comprising coal-tar coke and from 0.1 to 50 per cent of an oxid of lead.

14. A new article of manufacture having 110 a relatively low ignition temperature and a relatively high burning rate comprising coal-tar coke and a substance containing lead.

15. A new article of manufacture comprising 115 coke produced as the result of the complete distillation of coal-tar, said coke being characterized by the fact that it is sponge-like in structure, and non-crystalline, is dry, and when burned leaves a residue approximating two per cent composed of non-combustible matter and mineral ash; and a substance containing a metal acting as a combustion catalyst.

16. A new article of manufacture comprising 125 coke produced as the result of the complete distillation of coal-tar, said coke being characterized by the fact that it is sponge-like in appearance, and non-crystalline, is dry, and when burned leaves a residue approximating two per cent composed of 130

non-combustible matter and mineral ash; and a metal compound which catalyzes the combustion reaction.

17. A new article of manufacture comprising coke produced as the result of the complete distillation of coal-tar, said coke being characterized by the fact that it is sponge-like in appearance, and non-crystalline, is dry, and when burned leaves a residue approximating two per cent composed of non-combustible matter and mineral ash; and a metal oxide combustion catalyst.

18. A new article of manufacture comprising coke produced as the result of the complete distillation of coal-tar, said coke being characterized by the fact that it is sponge-like in appearance, and non-crystalline, is dry, and when burned leaves a residue approximating two per cent composed of non-combustible matter and mineral ash; and from 0.1 to 50 per cent of a metal oxide catalyst.

19. A new article of manufacture comprising coke produced as the result of the complete distillation of coal-tar, said coke being characterized by the fact that it is sponge-like in appearance, and non-crystalline, is dry, and when burned leaves a residue approximating two per cent composed of non-combustible matter and mineral ash; and an oxid of lead.

20. A new article of manufacture comprising coke produced as the result of the complete distillation of coal-tar, said coke being characterized by the fact that it is sponge-like in appearance, and non-crystalline, is dry, and when burned leaves a residue approximating two per cent, composed

of non-combustible matter and mineral ash; and from 0.1 to 50 per cent of an oxid of lead.

21. A new article of manufacture comprising coke produced as the result of the complete distillation of coal-tar, said coke being characterized by the fact that it is sponge-like in appearance, amorphous, and non-crystalline, is dry, and when burned leaves a residue approximating two per cent composed of non-combustible matter and mineral ash and a substance containing lead.

22. The process of treating carbonized material to depress its ignition temperature and increase its burning rate comprising incorporating therewith a substance containing a metal which serves as a catalyst for the combustion.

23. The process of treating carbonaceous material to depress the ignition temperature and increase the burning rate of its carbonized product comprising adding thereto a metal compound as a catalyst for the combustion, and carbonizing the mixture.

24. The process of treating carbonized material to depress its ignition and increase its burning rate comprising adding thereto a metal oxide which serves to catalyze the combustion reaction.

25. The process of treating carbonized material to depress its ignition temperature and increase its burning rate comprising incorporating therewith an oxid of lead.

In testimony whereof we have signed our names to this specification.

IRA H. DERBY.  
CARLETON B. EDWARDS.